

## 1

3,379,643

**FLEXIBLE MAGNETIC PLASTIC COMPOSITION**  
Richard R. Merkel, Hackensack, N.J., assignor to Allied  
Chemical Corporation, New York, N.Y., a corporation  
of New York  
No Drawing. Filed Nov. 27, 1964, Ser. No. 414,433  
6 Claims. (Cl. 252—62.54)

**ABSTRACT OF THE DISCLOSURE**

The invention more specifically relates to new and improved highly flexible high magnetic strength compositions comprising a highly specific high molecular weight chlorinated polyethylene having chlorine content between 33-55% by weight, less than 3% residual polyethylene crystallinity and intrinsic viscosity between 3 to 6 in o-dichlorobenzene at 100° C., together with at least 30 parts of normally liquid plasticizer per 100 parts of the chlorinated polyethylene, and at least about 90% by total weight of fine magnetic particles having size less than about 10 microns.

The invention relates to plastic compositions and more particularly to synthetic plastic compositions having magnetic strength.

The combination of magnetic particles with a resinous binder enables the production of materials having both flexibility and magnetic strength. Such flexible magnets are of increasing interest for use in special applications such as door closure gaskets and, more particularly, because of their potential as a replacement for the more expensive and rigid metallic magnets used, for example, in electric motors. To improve efficiency and expand the application of the flexible magnets there is continued interest in providing plastic compositions containing more and more amounts of magnetic material and having correspondingly higher magnetic capacity. However, the provision of plastic magnets of high magnetic strength is not an easy matter as the product must have other properties which unfortunately are severely depreciated by the presence of increased amounts of magnetic material. Notably among such properties is flexibility which can become so poor that cracking will be found on a single bending of a thin strip of the product. Thus, when attempting to produce a strength flexible magnet containing about 90% magnetic material it has been found in the past that even thin strips of such compositions would crack on bending well before reaching an angle of 90°. Further increase in magnet content have been found to produce compositions which are not capable of sustaining even a 45° bend without cracking. Such low flexibility not only reduces the attractiveness of the product but also renders manufacture and handling difficult without high scrap loss due to cracking. Further, a major economic advantage of the plastic magnets rests basically in the ability to form or shape by molding or extrusion procedures, in contrast to the more expensive manufacturing operations required for the metallic magnets. Consequently, ability to process the high magnetic compositions by such conventional plastic forming techniques is also of major importance.

An object of the present invention is to provide new and improved filled plastic compositions combining high flexibility and high magnetic strength.

Another object is to provide new and improved flexible magnets of high magnetic strength sufficient for use in applications where metallic magnets have been employed.

Other objects and advantages will be evident from the following description of the invention.

In accordance with the invention it has been found

## 2

that plastic composition of exceptionally high flexibility and magnetic strength is provided by combining fine magnetic particles with a highly specific chlorinated ethylene polymer which has been modified by addition of a normally liquid plasticizing material, the composition of the invention comprising: (A) 100 parts by weight of a chlorinated linear ethylene polymer having a chlorine content between about 33-55% by weight, less than 3% crystallinity as determined by differential thermal analysis, a glass transition temperature ranging from about minus 18° C.  $\pm$  10° C. for the 33% chlorine content chlorinated polyethylene up to about 63° C.  $\pm$  15° C. for the 55% chlorine content chlorinated polyethylene, and high molecular weight corresponding to an intrinsic viscosity between 3 to 6 in o-dichlorobenzene at 100° C.; (B) at least 30 up to about 130 parts by weight, preferably 40-70 parts, of a normally liquid plasticizer for said chlorinated polyethylene; and (C) at least 1400 parts by weight of fine magnetic particles. The compositions provided by this invention contain at least about 90% by weight of magnetic material and at such levels exhibit excellent flexibility as evidenced by bending through angles greater than 90°. It has been also discovered that further increasing the magnetic particle content above about 92-93% by weight results in compositions in which flexibility remains at a high level and is even improved over compositions containing less amounts of magnetic material. Hence, by the present invention it is possible to produce highly flexible magnetic compositions having magnetic particle content up to 95% by weight, or even more. In addition to high magnetic strength and flexibility the compositions of the present invention also combine good properties in general including good impact resistance, elongation, and tensile strength. The compositions may also be readily processed in conventional apparatus.

The compositions of the invention are based on a specific chlorinated polymer of ethylene having between about 33-55% by weight chemically combined chlorine and high molecular weight corresponding to an intrinsic viscosity of at least about 3 up to 6 in o-dichlorobenzene at 100° C. The more preferred chlorinated polyethylenes have a chlorine content between about 35-50% and an intrinsic viscosity between about 3.5 to 5. The chlorinated polyethylenes employed in the invention are also characterized by having certain chlorine distribution on the basic polyethylene chain such that the chlorinated polymers have little or no crystallinity as determined by differential thermal analysis, the crystallinity of the polymers being less than about 3%, preferably 0% crystallinity. The chlorinated polyethylenes also have definitive glass transition temperatures varying with chlorine content of the polymers. The glass transition temperatures of the chlorinated polyethylenes employed in the invention range from about -18° C.  $\pm$  10° C. for the 33% chlorine content chlorinated polyethylene up to about 63° C.  $\pm$  15° C. for the chlorinated polymers having 55% by weight chlorine. The more preferred chlorinated polyethylenes have glass transition temperature ranging from about -15° C.  $\pm$  10° C. for the 35% chlorine content chlorinated polyethylene up to about 35° C.  $\pm$  15° C. for the 50% chlorine content chlorinated polyethylene. The chlorinated polymers employed in the present invention are also those prepared by chlorination of a linear, high density polyethylene. The terms "linear" or "substantially linear," as used herein in the appended claims, shall mean a polyethylene characterized by high density and at most only nominal short chain branching in the form of methyl groups, usually less than about 10 methyl groups per 1,000 carbon atoms in the molecule, more commonly 0 to 5 methyl groups per 1,000 carbon atoms.

The chlorinated polyethylenes by themselves will not

accept the large amounts of magnetic particles required to form the compositions of the invention. In order to obtain compositions of high magnetic strength it is necessary to blend the chlorinated polyethylene with a plasticizing material which is a liquid under normal conditions. It has also been found that certain liquid plasticizers which are also surfactants, i.e. have surface active properties, will produce a substantial improvement in both magnetic strength and flexibility of the plastic magnets having a given amount of magnetic particles.

The amount of plasticizer required to be effective is at least about 30 parts ranging up to about 120 parts per 100 parts of the chlorinated polyethylene. The more preferred compositions contain about 40 to 70 parts of plasticizing material. The plasticizer employed in the composition is normally liquid material and plasticizers of this type are well known. Such plasticizers include, by way of example, the chlorinated aliphatic and aromatic hydrocarbons, the liquid epoxy resins such as those prepared by reaction of epichlorohydrin and bisphenol A, the epoxidized drying oils such as epoxidized soya bean oil and the monomeric and polyester plasticizers. The chlorinated hydrocarbons useful in the compositions of the invention have chlorine content generally between about 20% to 70% by weight and low molecular weight between about 200 to 4000. The more preferred chlorinated hydrocarbon plasticizers are the normally liquid chlorinated aliphatic hydrocarbons having chlorine content between about 30% to 55% and molecular weight between about 200 to 2000. The monomeric ester plasticizers are generally preferred and include those formed from the acids such as phosphoric, phthalic, adipic, sebacic, etc. Suitable alcohols for forming the monomeric esters have generally 2 to 16 carbon atoms, more usually 4 to 12 carbons. Examples of such monomeric plasticizers include tricresyl phosphate, diethyl phthalate, dibutyl phthalate, 2-ethylhexyl phthalate, diethyl phthalate, butyl-cyclohexyl phthalate, didecyl phthalate, diisodecyl phthalate, diisobutyl phthalate, octyl decyl phthalate, diamyl phthalate, dicapryl phthalate, diethoxyethyl phthalate, dibutoxyethyl phthalate, diethyl isophthalate, diethyl adipate, and dibutyl sebacate. Generally, the more preferred plasticizers are the monomeric esters of phthalic acid. Certain liquid plasticizers are also known to have surface active properties and such materials have been found exceptionally beneficial in producing magnetic compositions combining both high magnetic strength and flexibility at a given loading at magnetic particles. Very suitable plasticizers of the surfactant type are the fatty acid esters of alcohols having 2 to 12 carbon atoms, preferably 3 to 8 carbon atoms. A specific example of such a fatty acid ester is butyl stearate. The surfactant plasticizers are employed in combination with the more conventional plasticizers and as little as about 2 parts per 100 parts of chlorinated polyethylene is effective in obtaining improved properties. The surfactant plasticizers may be employed in amounts representing between about 2-85% by weight of the total plasticizing materials with best results obtained when the surface active materials represent between about 30-75% of the total plasticizer. The surface active plasticizers are especially effective at the higher magnetic loading contents above about 92-93% where the association between the chlorinated polyethylene binder and magnetic particles becomes a critical factor obtaining both high flexibility and magnetic strength.

The chlorinated polyethylenes employed in practice of this invention are not readily or satisfactorily plasticized by conventional procedures at or about room temperatures. In preparation of the compositions this problem may be overcome by incorporation of the plasticizer for the chlorinated polyethylene at an elevated temperature about about 200° F. but not in excess of about 430° F. At such temperatures the chlorinated polyethylene will readily accept the plasticizing material and form therewith a composition of especially good homogeneity and

also high flexibility and magnetic filler and loading content. The chlorinated polyethylene is subject to decomposition and thermal degradation at the higher temperatures and therefore it is desirable to first admix the chlorinated polyethylene with a heat stabilizer to protect the polymer against degradation as it is subsequently heated to the plasticizing temperatures. The heat stabilizers employed may be those well-known materials commonly used with the chlorine-containing resins. Examples of such stabilizers include the inorganic salts and organic complexes of salts and metals such as barium, cadmium, tin, zinc, lead, sodium, etc. Also suitable are the liquid epoxy resins such as those prepared by reaction of epichlorohydrin and bisphenol A. The stabilizing materials also serve to protect the polymer during subsequent extrusion, molding or other forming operations conducted at elevated temperatures. The amount of heat stabilizer added is usually between about 1 to 15 parts to 100 parts of the chlorinated polyethylene, more usually between about 2 to 10 parts. Admixing of the plasticizing material at elevated temperatures is satisfactorily accomplished in conventional compounding apparatus, for example, a Banbury mixer or rubber roll mill. Heating of the chlorinated polyethylene during mixing may be accomplished by supplying heat through the mixing apparatus and/or the frictional heat of the mixing operation. The plasticizer may be initially admixed with the chlorinated polyethylene at room temperature or at elevated temperatures on the mixing apparatus either before or after the chlorinated polyethylene is heated to the desired elevated temperature. It is generally preferred in obtaining best results and efficient operation to rapidly heat the plasticizer and chlorinated polyethylene to the plasticizing temperature within a short period of about 5 minutes, preferably less than 3 minutes. This may be suitably accomplished by pre-heating of the mixing apparatus and/or chlorinated polymer above about 150° F. According to a preferred procedure the plasticizer is premixed with the chlorinated polyethylene and heat stabilizer in separate pre-mixing equipment and the resulting premix charged to the mixing apparatus, preferably a two roll rubber mill which has been preheated to a temperature near or above the plasticizing temperature, preferably between about 200° F. to 350° F. The plasticizing material is then readily combined with the chlorinated polyethylene above the plasticizing temperature and a homogeneous mass is found in a matter of minutes, usually between 1 to 10 minutes after charging to the mixing apparatus. The magnetic particles are then admixed with the resulting plasticized chlorinated polyethylene composition, preferably after adjusting the temperature of the mass to a reduced temperature between about 150-220° F. It has been found desirable when producing the highly filled magnetic compositions to add the magnetic particles in stages. For example, a preferred procedure involves the addition of a major portion but not all of the magnetic particles. After thorough mixing of the first charged particles the balance of the magnetic material may be added and mixing continued to form a homogeneous product. Such procedure aids in distribution of the magnetic particles in the binder and is also a factor in obtaining the combination high flexibility and magnetic strength. Another preferred method involves addition of the magnetic particles prior to heating of the polymer to the plasticization temperature to take advantage of the frictional heat generated by mixing of the solid filler material. The heat-stabilized chlorinated polyethylene with or without the plasticizer is charged to a two roll mill which is preferably preheated to a temperature above about 150° F. usually between 180-230° F. After about 1-2 minutes mixing of the chlorinated polymer with the plasticizing material the magnetic particles are added, preferably in stages. Heat generated by mixing of the magnetic particles facilitates the rise in temperature of the mass such that the plasticizing temperature is reached within a short time and plasticization and formation of the filled composition readily

obtained. In this procedure cooling of the mixing apparatus is recommended as by the use of ordinary water to control the temperatures below about 470° F. The composition sheeted out from the mill is especially suitable for extrusion, molding or other forming operations to produce a variety of flexible products. The magnetic material employed may be any of the well-known finely divided permanently magnetizable materials, it being also understood that the term "magnetic" may also mean magnetizable in view of the practical requirements of magnetizing the particles after combination with the binder. In the compositions the magnetic filler will have particle size ranging from about 0.5 to 15 microns with average particle size preferably between about 1 to 3 microns. The more preferred magnetic fillers are those complex metal oxides well-known as "ferrites" which term, as used herein, designates an inorganic material of the formula  $MFe_mO_n$  wherein M is a divalent metal and m and n are whole numbers. The more preferred metal ferrites are the barium ferrites, for example, the barium ferrites represented by the formula  $BaFe_{12}O_{19}$ .

The chlorinated polyethylene is desirably prepared for use in the invention by chlorination of high molecular weight linear polyethylene in a heterogeneous medium in stages defined by introduction of chlorine at a temperature first below and then above the crystalline melting point of the polymer, as described in copending application of Pisanchyn et al., Ser. No. 86,309, filed Feb. 1, 1961, now abandoned. Preparation of the chlorinated polyethylene is most desirably accomplished by two-stage suspension chlorination of the linear, high molecular weight polyethylene with first-stage chlorination being carried out in aqueous slurry at temperature below the crystalline melting point of the ethylene polymer, preferably at a temperature of about 60° C. to 130° C., more usually at 90-120° C., until at least about 5 percent, preferably about 10 percent, of chlorine has been introduced into the polymer. In the second stage the chlorination is continued in the aqueous slurry at a temperature above the crystalline melting point of the polymer but below the softening point of the chlorinated outer coating thereof until the desired chlorine is added. Second-stage chlorination temperatures are of the order of at least about 135° C. and preferably lie in the range of about 135° C. to 150° C. If desired, chlorination in the second-stage may be carried out at a temperature above the crystalline melting point of the polymer for time sufficient to add at least about 5 percent chlorine by weight, preferably until at least a total of 25% chlorine is added to the polymer, and the chlorination then continued at a lower temperature, e.g. 110° C. to 120° C., until the desired total chlorine is added.

The suitable chlorinated polyethylenes are derived from a linear polymer of ethylene having a molecular weight of at least about 700,000 ranging up to about 5,000,000, preferably between about 1,000,000 to 3,000,000. Chlorination of the linear polyethylene of 1-5 million molecular weight by the subject two-stage process will produce the particularly preferred chlorinated polyethylenes having 33-55% by weight chlorine and high molecular weight corresponding to an intrinsic viscosity within the range of at least about 3.5 in o-dichlorobenzene at 100° C. These preferred chlorinated polyethylenes are also chemically inert and insoluble at 20-25° C. in organic solvents such as esters, acids and alcohols. They have tensile strength values according to ASTM Method D 638-58T (at drawing rate of 2 inches per minute) of at least about 2,500 p.s.i., usually between about 2,500 p.s.i. and about 4,500 p.s.i. The chlorinated polyethylenes also have true ultimate tensile strengths according to ASTM Method D 638-58T of at least about 11,000 p.s.i., with the preferred materials of 35-50% chlorine content having true ultimate tensile strength values between about 11,000 to 20,000. The chlorinated polyethylenes have less than about 3% crystallinity by differential thermal analysis, preferably 0% crystallinity, and also are characterized by low glass transition temperatures ranging from about minus 18° C.  $\pm 10°$

C. for the 33% chlorine material up to about 63° C.  $\pm 15°$  C. for the 55% chlorine material. The preferred chlorinated polyethylenes have glass transition temperatures at least as low as about minus 15° C.  $\pm 10°$  C. for the 35% chlorine material ranging to about 35° C.  $\pm 10°$  C. for the 50% chlorine content chlorinated polyethylene. The glass transition temperatures, a second order transition temperature, can be determined by plotting the stiffness modulus of the samples as a function of temperature, and can be defined as the temperature at which the stiffness modulus of the sample possesses a value of  $1.45 \times 10^4$  p.s.i. or  $10^9$  dynes/cm.<sup>2</sup>. The determination may be made in accordance with ASTM Test D1053-61. In effect, the glass transition temperature is that temperature below which the chlorinated polymers become brittle. Above the glass transition temperature the polymers become more flexible and rubbery. The low glass transition temperatures of the chlorinated polyethylenes contribute to the ability of the compositions of the invention to retain good elastomeric properties at low temperatures.

For preparation of the chlorinated polyethylene a particularly suitable linear high molecular weight polyethylene which may also be characterized by containing long chain polyethylene branches is produced, as described in British Patent 858,674 of June 11, 1961 to Allied Chemical Corporation, by gas phase polymerization of anhydrous, oxygen-free ethylene below the softening point of the polyethylene over a porous, frangible catalyst of an inorganic compound of chromium and oxygen and an active metal alkyl on a support of the group consisting of silica and silica-alumina. The polyethylenes produced thereby contain residue of the chromium-silica catalyst systems dispersed throughout the polyethylene is an amount of at least about .001%, usually .001-.002%, by weight. The chromium-silica catalyst material added during polymerization is retained in the polyethylene during chlorination and contributes to the properties of the chlorinated polyethylene. Prior to chlorination the polyethylene from which the chlorinated polyethylene is derived has a density between about 0.935 and about 0.985 and a crystallinity of at least 75%, and customarily in the range of 75% to 85%, as determined, for example, by differential thermal analysis. The preferred polyethylenes produced by British Patent 858,674 have weight average molecular weight between 1.0 million and about 5.0 million, preferably between 1.0 to 3.5 million, as calculated according to the method of P. S. Francis et al. from the viscosity of about 0.05 to 0.1 gram per 100 cc. solution in decalin at 135° C. using the equation:

$$n = 6.77 \times 10^{-4} M^{0.67}$$

where

$n$ =intrinsic viscosity

$M$ =weight average molecular weight (J. Polymer Science, vol. 31, pp. 453-466, September 1958)

The following examples in which parts and percentages are by weight demonstrate the practice and advantages of the present invention.

#### Examples 1-6

Chlorinated polyethylene of 45% chlorine was prepared by staged aqueous chlorination of linear polyethylene having a weight average molecular weight of about 1.5 million and density of 0.94. The polyethylene employed was prepared in accordance with British Patent 858,674 (Example 6) by gas phase polymerization of anhydrous oxygen-free ethylene over a catalyst of magnesium dichromate on a porous support with aluminum triisobutyl. The support was composed of 90% silica and 10% aluminum. Chlorination of the polyethylene in a first stage was carried out at a temperature of about 100° C. until 17% chlorine was added to the ethylene polymer followed by second stage chlorination at a tempera-

ture of 140° C. until a total of about 35% chlorine was added. Chlorination was then continued at a temperature of about 110–120° C. until a total of 45% by weight chlorine was added. The chlorinated polyethylene recovered from the slurry was washed and dried overnight at a temperature of 60° C. The chlorinated polyethylene had a glass transition temperature of about 5° C. (ASTM D1053–63) and 0% crystallinity as measured by differential thermal analysis. The chlorinated polyethylene also had high molecular weight corresponding to an intrinsic viscosity of 4.0 in o-dichlorobenzene at 100° C.

A series of magnetic compositions was prepared by the following procedure from the above prepared chlorinated polyethylene. 100 parts of the chlorinated polymer was admixed with 3 parts of a barium-cadmium organic heat stabilizer obtained from the National Lead Company under the trademark "Temex" 5C. There was also added about 58 parts of dioctyl phthalate as plasticizer and about 0.5 part of stearic acid as lubricant. Each of the compositions contained barium ferrite as magnetic filler in varying amounts between about 1400 to 2400 parts by weight. The barium ferrite had an average particle size of about 1–2 microns. In preparing each of the compositions between about 90–95% of the total barium ferrite was added and the resulting components charged to a two roll (6 inch x 12 inch) differential speed rubber mill which had been preheated to a temperature of about 300° F. by internal steam heating of the two mill rolls. After about two minutes on the mill the temperature of the mixture was increased to about 300° F. and fluxed. Mixing of the charge was then continued for an additional 5–10 minutes during which a homogeneous mass was formed. The temperature of the mixture was then reduced to about 180° F. over the course of about 10 minutes and there was then added to the mixture the remaining 5–10% of barium ferrite. Mixing on the mill was then continued for an additional 3–5 minutes to form a homogeneous mass which was sheeted out from the mill to form sheets of 0.14 inch thickness. Specimens of each of the compositions were then evaluated and the results are tabulated below in Table I.

TABLE I

| Example No.                                      | 1     | 2     | 3     | 4     | 5     | 6     |
|--------------------------------------------------|-------|-------|-------|-------|-------|-------|
| Barium Ferrite, Parts by weight                  | 1,449 | 1,628 | 1,740 | 1,890 | 2,000 | 2,316 |
| Barium Ferrite, percent by weight                | 90    | 91    | 91.5  | 92    | 92.5  | 93.5  |
| Specific Gravity                                 | 3.80  | 3.90  | 3.90  | 3.93  | 3.93  | 3.88  |
| Crack Angle <sup>1</sup>                         | >90   | >90   | 86    | 66    | 51    | 59    |
| Mandrel Bend, 1 inch mandrel                     | 180   | 180   | 180   | 180   | >60   | >60   |
| Magnetic Strength at 0.015 inch gap <sup>2</sup> | 0.221 | 0.238 | —     | 0.256 | 0.229 | —     |

<sup>1</sup> Determined with 2 inch specimen on Tinius Olsen Stiffness Tester at 50 load dial reading employing a 0.995 pound calibrating weight. Maximum angle obtainable in stiffness tester is 90°.

<sup>2</sup> Lbs. lift per inch length.

Table I shows the compositions of the invention to have high magnetic strength and flexibility. The compositions of Examples 1–4 inclusive containing up to 92% by weight barium ferrite all sustain a full 180° bend around a 1 inch mandrel. The compositions of Examples 5 and 6 containing substantially greater amounts of barium ferrite resist cracking after bending under load through an angle of at least 50° in the Olsen Stiffness Tester. The composition of Example 1 was further evaluated and found to have a tensile strength of 700 p.s.i. and unusually good elongation of 85%.

#### Examples 7–10

A series of four additional compositions were prepared employing components and procedure similar to Example 1 except that the plasticizing material was a combination of 23 parts dioctyl phthalate and 30 parts butyl stearate. These compositions were then evaluated

as in Examples 1–6 and the results are tabulated below in Table II.

TABLE II

| Example No.                                      | 7     | 8     | 9     | 10    |
|--------------------------------------------------|-------|-------|-------|-------|
| Barium Ferrite, parts by weight                  | 1,503 | 1,689 | 1,921 | 2,219 |
| Barium Ferrite, percent by weight                | 90    | 91    | 92    | 93    |
| Specific Gravity                                 | 3.83  | 3.93  | 4.00  | 4.00  |
| Crack Angle <sup>1</sup>                         | >90   | >90   | 50    | >90   |
| Mandrel Bend, 1 inch mandrel                     | 180   | 180   | 135   | 180   |
| Magnetic Strength at 0.015 inch gap <sup>2</sup> | 0.221 | 0.229 | 0.247 | 0.265 |

<sup>1</sup> Determined with 2 inch specimen on Tinius Olsen Stiffness Tester at 50 load dial reading employing a 0.995 pound calibrating weight. Maximum angle obtainable in stiffness tester is 90°.

<sup>2</sup> Lbs. lift per inch length.

15 The Table II compositions all have excellent flexibility and high magnetic strength which increases approximately proportionately with the amount of magnetic particles. Table II also clearly demonstrates the ability of the compositions of the invention to exhibit improved flexibility along with high magnetic strength upon increase of the amount of magnetic particles above about 92%. Hence, the composition of Example 9 containing 92% magnetic particles has a crack angle of 50° and mandrel bend of about 135° while the composition of 20 Example 10 containing some 300 parts more of the particles has substantially improved flexibility with a crack angle greater than 90° and flexibility around the 1 inch mandrel of 180°. The Table II also clearly demonstrates the effectiveness of the butyl stearate in improving magnetic strength, particularly at the higher contents of magnetic particles. Hence, the composition of Example 10 containing 93% magnetic material has superior magnetic strength and also flexibility over the composition of Example 6 containing 93.5% magnetic particles.

25 30 35 Although certain preferred embodiments of the invention have been disclosed for purpose of illustration, it will be evident that various changes and modifications may be made therein without departing from the scope and spirit of the invention.

40 I claim:

45 1. A highly flexible highly magnetic plastic composition comprising a binder of a chlorinated linear polymer of ethylene and at least 30 parts up to about 130 parts of a normally liquid plasticizer per 100 parts of the chlorinated polyethylene and at least about 90% by weight of fine magnetic particles having size less than about 10 microns, said chlorinated polyethylene having a chemically combined chlorine content between 33–55% by weight, less than 3% crystallinity as determined by differential thermal analysis, glass transition temperature ranging from about minus 18° C. ± 10° C. for the 33% chlorine content chlorinated polyethylene up to about 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345

35° C.  $\pm$  15° C. for the 50% chlorine content chlorinated polyethylene, and molecular weight corresponding to an intrinsic viscosity between about 3 to 6 o-dichlorobenzene at 100° C.

5. The composition of claim 4 in which the amount of liquid plasticizer is between about 40-70 parts of which between about 30-75% by weight is a fatty acid ester of an alcohol of 2-12 carbon atoms.

6. The composition of claim 4 in which the liquid plasticizer is a mixture of a phthalate plasticizer and between about 30-75% parts by total plasticizer weight of butyl stearate.

## References Cited

## FOREIGN PATENTS

1,323,095 2/1963 France.

## OTHER REFERENCES

Kresser: Polyethylene, 1957, p. 64.

Penn: PVC technology, 1962, pp. 73-76, 98 and 170-171.

10 TOBIAS E. LEVOW, Primary Examiner.

ROBERT D. EDMONDS, Examiner.